

# UNITED STATES PATENT OFFICE.

EMILE BRONNERT, OF MÜLHAUSEN, ALSACE-LORRAINE, FRANCE.

## MANUFACTURE OF VISCOSE SILK.

1,376,672.

Specification of Letters Patent.

Patented May 3, 1921.

No Drawing.

Application filed September 10, 1920. Serial No. 409,441.

To all whom it may concern:

Be it known that I, EMILE BRONNERT, a citizen of the Republic of France, residing at 1 Quai du Barrage, Mülhausen, Alsace-Lorraine, France, have invented certain new and useful Improvements in the Manufacture of Viscose Silk, of which the following is a specification.

It is known that raw viscose can be spun 10 in diluted sulfuric acid to lustrous threads, if measures be taken to insure the reaction proceeding properly.

While younger viscose may only be spun with caution in weaker acid, older viscose 15 must be spun in stronger acid which is also warm.

Now it has been found that in order to obtain a thread of extreme fineness, the acid concentration and with it the precipitating 20 power of the bath must be all the stronger the thinner the individual thread to be obtained is desired to be. With a bath of pure diluted sulfuric acid or sulfuric acid with for instance as much sulfate of sodium as is 25 ultimately present in the bath when spinning as a condition of equilibrium or also with salts of other bases and acids, the individual thread strengths of titrations which can be obtained with determined sulfuric 30 acid baths, act in relation to each other in a manner approximately inverse to the squares of the sulfuric acid concentrations of the baths. On spinning very fine threads according to the usual method of operation it 35 is, therefore, essential to use a relatively high sulfuric acid concentration of the bath. With so strong an acidity of a bath containing a small percentage of salts, it is, however, with the normal viscose of about 8% 40 cellulose and 7% caustic soda content only possible to spin a relatively well ripened viscose if technically useful lustrous products are to be obtained.

With the many dangers of practical spinning it is, however, desirable that the composition of the precipitating bath be as independent as possible of the ripeness of the viscose. So far assistance in this connection has mostly been obtained in that, larger 45 quantities of salts were added to the bath. Now it has been found that the proportion of the degree of ripeness of the viscose to the acid concentration can be changed in a far reaching manner without prejudice to the luster and fullness of the product, if

certain quantities of oxy-acid be added to the sulfuric acid, especially lactic acid.

Such baths, which customarily are mostly used warm, are especially valuable for draw spinning of cellulose hydrate threads, which 60 are insoluble in water, from the usual spinning openings of 0.1 mm. diameter. However, with such solutions, attention must be given not only to the sulfuric acid concentration at the time of precipitating the 65 threads, but also to a regular feed of spinning solution corresponding to the simultaneous number and the titer of the threads desired at the time to form a collective thread and also to the speed of drawing off, both of 70 which latter factors determine the consumption of spinning solution.

It is preferable to increase the quantity of lactic acid, the younger the viscose to be used.

To appreciate the peculiar effect of the new process a comparison of Examples I and V with the other examples may be had.

### Example I.

In a warm bath of 45° with 135 gr. sulfuric acid per liter, there is introduced 80 through nozzles of about 0.10 mm. diameter, the usual raw viscose of about 8%, relatively young, of say about 9° ripeness 85 (chlorid of ammonium standard). The threads of about 7 deniers rising from the bath with a speed of about 45 m. are at once washed and then treated further in the usual manner.

The finished product does not present anything worthy of remark.

The threads have a more or less round elliptic cross section.

### Example II.

A sulfuric acid bath of the same character as used in Example I is mixed with 95 10 gr. lactic acid per liter, that is to say, with a catalytic quantity only and the same viscose is spun in in the same manner.

The spinning takes place with extreme smoothness, and without any breakage of the threads.

The washed and finished dry thread presents a coarse toothed more or less bean-shaped cross section, such as shown by threads which have been spun in acid which contained quantities of salt exceeding the proportion of bisulfate.

110

*Example III.*

A sulfuric acid bath of 135 gr. sulfuric acid per liter, but otherwise similar to that employed in Example I, is mixed with 50 gr. lactic acid per liter and the same raw viscose of 9° ripeness (chlorid of ammonium standard) is again introduced into the bath. The spinning process action is almost perfect. The final product shows in cross section forms similar to those obtained by Example II, only the toothing or dentation is somewhat less and coarser, the softness and luster of the product are on the other hand quite prominent so that it equals the best products from acid baths which contain much salt, in fact is even superior to them. The elasticity of the threads increases with the increasing lactic acid content of the bath.

Whether the lactic acid is able to force back the free ions of the sulfuric acid similar to the salts forming bisulfates need not be discussed. The effect is at all events a most peculiar one.

This is brought out in a marked manner by a comparison of the results illustrated in Examples IV and V.

*Example IV.*

Young viscose, this time of 12° ripeness, with a spinning length of 20 cm. is spun as stated in the other examples into a 45° warm spinning bath of 135 gr. sulfuric acid and 50 gr. lactic acid per liter. There is again produced with great certainty a directly washable thread which after finishing, is of very fine luster and of remarkable softness, body and elasticity.

*Example V (to illustrate prior art.)*

If on the contrary the same young viscose of 12° ripeness is spun in the same manner in warm sulfuric acid of 135 gr. per liter without the addition of lactic acid, then only a much duller and much thinner thread than those produced by the processes described in Examples II to IV, is obtained even if the bath has been enriched up to the same equilibrium of about 100 to 120 gr. sodium sulfate per liter.

The lactic acid is therefore to a pronounced extent quantitatively different from the action of the sulfate; the presence of sulfates and other salts, however, is not disturbing. It does not itself appear to have any actual precipitant action as a thread former, it requires the coöperation of salts or acids.

If, as already proposed a spinning bath be used of a sodium lactate solution with an addition of about 140 gr. lactic acid per liter, then only a water soluble thread is obtained which must be subsequently fixed by mineral acid or the like.

If as much of the uni-basic lactic acid per liter of water be taken as would be equivalent to the acidity of 100 gr. sulfuric acid that is to say about 200 gr. water free lactic acid per liter, then no thread formation takes place when a raw viscose solution of 9° ripeness is pressed in.

Also when viscose of 9° ripeness is allowed to flow into a heated spinning bath of about 180 gr. anhydrous lactic acid and 90 gr. sulfuric acid per liter, then threads of 7.5 deniers can hardly be spun.

Viscose can only be spun to directly washable threads when the sulfuric acid content of the spinning bath is increased to 115 gr. per liter. It is therefore demonstrated that the lactic acid is substantially without influence upon the thread formation, as the viscose in question can also be spun just as smoothly although not of the same quality in sulfuric acid alone of 115 gr. per liter.

These sulfuric acid and oxy-acid baths, and especially such with lactic acid, are pre-eminently and quite suitable for the production of fine and ultra-fine threads, of course as well for instance for threads of ordinary caliber.

The described draw-spinning process is particularly suitable and yields a very fine fluff free product.

The friction of the threads on the spinning bath particles is apparently reduced to a minimum. The sodium sulfate, which reaches a condition of equilibrium, has no harmful effect at all, and does not crystallize upon the threads, as this is in any case prevented by the simultaneous formation of deliquescent sodium lactate.

I claim:

1. A spinning bath for use in the manufacture of viscose silk, containing sulfuric acid and lactic acid.

2. A spinning bath for use in the manufacture of viscose silk, containing sulfuric acid and lactic acid, the quantity of lactic acid being proportioned substantially inversely to the age of the viscose to be treated.

3. A spinning bath for use in the manufacture of viscose silk, containing sulfuric acid and lactic acid, the quantity of lactic acid being proportioned substantially inversely to the age of the viscose to be treated, and the sulfuric acid being proportioned to the fineness of the thread to be produced.

In witness whereof, I have hereunto signed my name in the presence of two subscribing witnesses.

EMILE BRONNERT.

Witnesses:

L. R. SALIE,  
N. SCHLUMBORGER.